

[54] COAL DERIVED/CARBON DIOXIDE FUEL  
SLURRY AND METHOD OF  
MANUFACTURE

[75] Inventors: Edmond G. Meyer, Laramie, Wyo.;  
Lee G. Meyer, Englewood, Colo.

[73] Assignee: Carbon Fuels Corporation,  
Englewood, Colo.

[21] Appl. No.: 651,947

[22] Filed: Sep. 19, 1984

**Related U.S. Application Data**

[63] Continuation-in-part of Ser. No. 427,937, Sep. 29, 1982,  
Pat. No. 4,475,924, which is a continuation-in-part of  
Ser. No. 247,382, Mar. 24, 1981, abandoned.

[51] Int. Cl.<sup>4</sup> ..... C10L 1/32

[52] U.S. Cl. ..... 44/51; 44/1 R;  
44/1 SR; 406/47

[58] Field of Search ..... 44/51, 1 R, 1 SR;  
406/47

[56]

**References Cited**

**U.S. PATENT DOCUMENTS**

|           |         |                     |          |
|-----------|---------|---------------------|----------|
| 4,030,893 | 6/1977  | Keller .....        | 44/1 SR  |
| 4,113,445 | 9/1978  | Gettert et al. .... | 48/197 R |
| 4,192,651 | 3/1980  | Keller .....        | 44/1 SR  |
| 4,208,251 | 6/1980  | Rasmussen .....     | 44/51    |
| 4,351,645 | 9/1982  | Marion et al. ....  | 48/61    |
| 4,490,156 | 12/1984 | Marion et al. ....  | 48/61    |

*Primary Examiner*—Jacqueline V. Howard  
*Attorney, Agent, or Firm*—Lee G. Meyer

[57]

**ABSTRACT**

Coal char produced by the pyrolytic destructive thermal distillation of coal in the absence of oxygen is ground, sized and then admixed in suitable portions with a liquid carbon dioxide to form a fluidic, liquid-solid mixture which is a transportation medium for a nonpolluting, stable, high energy solid fuel composition. The liquid organic fraction obtained from the low boiling fractions derived from the pyrolysis of coal is used as a feedstock or as a liquid hydrocarbon fuel.

19 Claims, No Drawings

## COAL DERIVED/CARBON DIOXIDE FUEL SLURRY AND METHOD OF MANUFACTURE

This application is a continuation-in-part of U.S. patent application Ser. No. 427,937 filed Sept. 29, 1982, now U.S. Pat. No. 4,475,924 issued Oct. 9, 1984, which is a continuation-in-part of U.S. patent application Ser. No. 247,382 filed Mar. 24, 1981, now abandoned.

### DESCRIPTION

#### Technical Field

The parent application which is incorporated in its entirety by reference by reference as if it were completely set out herein, discloses a transportable fuel system as well as completely combustible, transportable fuel compositions derived from coal, which compositions contain particulate coal char, and methods for making such a system. The parent application specifically discloses that the fuel system can be derived entirely by the pyrolysis of coal.

The instant invention relates to fluidic transportable fuel systems and fuel compositions, which fuel systems contain particulate coal char derived from solid carbonaceous fuels such as coal, lignite and lower rank coals, and the like slurried in liquid carbon dioxide. More particularly, this invention relates to high energy, non-polluting, transportable fluidic fuel systems and methods for making such systems. The transportable composition forms a fuel transport medium from which the particulate coal char is separated and used as a fuel for solid-fuel fired combustion devices.

The liquid organic material produced simultaneously with the particulate coal char is used as a liquid combustion fuel or as a feedstock. In a further aspect, as portion of the char is used as a combustion fuel prior to producing the transportable fuel system. Advantageously, char is admixed with a portion of the liquid organic material, preferably a higher boiling fraction, to enhance combustion characteristics and to reduce absorption of moisture by the char.

#### Background Art

In the U.S., there is fifteen times as much recoverable coal as recoverable oil and natural gas combined. Coal, therefore, should be the primary fuel for large stationary and mobile combustion installations and for production of process heat. Not only should America's energy needs increasingly be met by coal, but coal could also meet the need of other industrialized and developing countries. Coal could be America's answer to the "energy" balance of trade deficit. However, such is not presently the case.

Although 200 billion tons of economically recoverable coal, and an undetermined amount of coal which is not presently economically recoverable, are present in the United States (representing more than 70% of domestic fossil energy resources), coal currently supplies less than 20% of all of our energy production. A number of factors have combined to create this disparity. Even with the abundance of coal energy, it has not heretofore been competitive with, nor as easily utilized as, other fossil fuels such as oil, natural gas and the like.

One very effective use of our coal resources is in stationary plants producing electricity or process heat. Stationary power conversion facilities do not require high performance liquid and gaseous hydrocarbons. These fuels are better utilized in transportation and

5 certain residential/ commercial uses. However, the use of coal in stationary power facilities requires that either the solid be transported to the power facility or the power plant be constructed at the mine site for "mine mouth" utilization of the coal. Utilization at the mine site is not always an efficient method for producing electricity because of environmental problems, and electrical transmission losses. Yet, production of electrical energy at other than the mine site requires that the solid coal be transported to the power plant. Coal is currently shipped by rail in unit trains but the current rail capacity may be inadequate to move the tonnage required to replace existing use of more costly and scarce liquid and gaseous fuels. Moreover, the required handling of coal as a solid fuel is cumbersome, wasteful and expensive.

10 The greatest deterrent to full utilization, domestic and foreign, of the U.S.' coal resource is the nature of coal itself. First, raw coal is not a uniform combustion product. Second, as a solid it is difficult to handle and expensive to transport. Third, it contains organic sulfur and nitrogen, which, upon combustion, produce air pollutants which have been associated with acid rain. Fourth, it contains ash which, upon combustion produces pollutants and slag. In addition to the above problems, the majority of the energy transportation and combustion systems in this country revolve around oil and natural gas which are relatively uniform, pipeline transportable liquid and gaseous fuels. The coal transportation and quality problems are compounded by the fact that, although coal reserves are distributed throughout the U.S., coal from different reserves has a wide range of characteristics. Coals, even of the same rank, have different compositions. This limits the interchangeability of coal in combustion systems and thus increases expense and reduces markets. For example, intermountain Western coal, while low in sulfur, is also generally low in BTU per unit weight and has a high water content. Each type of coal requires different pollution control equipment and a specific boiler system. Coal of one region (or even of a particular mine) cannot be efficiently combusted in boilers designed for coal from another source. Therefore, coal is not as uniform a fuel as is, for example, #6 fuel oil.

15 The inefficient and expensive handling, transportation and storage of the solid material has made the conversion of oil-fired systems to coal less economically attractive. Liquids are much more easily handled, transported, stored and fired into boilers. Because of this nation's dependence on oil and natural gas, existing fuel transportation systems on the U.S., from pipelines to ocean-going tankers, are designed for liquids and gases.

20 Various methods, for the most part not economically viable, have been proposed for converting coal to synthetic liquid or gaseous fuels. Recently developed process technology permits the conversion of coal to synthetic liquid or gaseous fuels at the mine site. While this "synfuel" is more easily transported than coal, the conversion process is capital intensive and requires a great deal of water. The process is also very energy intensive in that essentially every carbon atom in the coal matrix is converted to a hydrocarbon. Despite the high processing costs, the resultant synfuel, like crude oil derived fuels, is valuable as a transportation fuel.

25 Methods for creating coal slurries or mixtures which facilitate liquid transport and fluidic firing into boiler systems have been proposed but have not been com-

pletely successful. To produce a slurry, raw coal is ground, sized, slurried with water or other liquid, and stabilized. The goal is to obtain a product which handles like a liquid, not only facilitating the transportation step itself, but also reducing labor costs and eliminating the many other handling problems of solids and reducing the capital costs required to convert oil-fired systems to use solid coal.

Coal slurries are comprised of ground coal particles which have jagged, nonsymmetrical shapes due to fracturing along crystal faces. This configuration not only is abrasive to conduit systems but also adversely affects the loading limits and flow characteristics of any resultant slurry. Since coal is the main fuel constituent in such slurries, furnace and stack modifications are still required in order to burn coals from different regions. Non-aqueous liquids used for slurring (including alcohol) tend to solubilize impurities in the coal. These impurities tend to combine with the liquid medium and form polymerized materials which "varnish" pipelines and alter rheology characteristics.

Previous coal slurries have required special pipelines and pumping equipment. Aqueous coal slurries have additional drawbacks: (1) The water which is necessary to slurry coal is in short supply for coal reserves in the intermountain West. (2) Water must be removed from the slurry and the coal must be dried prior to introduction of the fuel into a furnace or boiler to avoid incurring a substantial heat penalty. (Derating of the boiler) (3) Dewatering and disposal of the slurry water creates a pollution problem.

Liquids other than water, such as alcohol or liquid carbon dioxide, may be used as the slurring liquid but are expensive and usually require water for manufacture or utilization of cryogenic handling and pipeline systems. In addition to being abrasive, coal slurries tend to settle upon standing, thereby causing flow problems in pipelines and ballast problems aboard ships.

While coal/water slurries and coal/alcohol slurries require substantial system modification in order to be fired in existing oil-fired combustion systems, coal/oil mixtures ("COM") are able to be burned in existing coal-fired furnaces, boilers and process heat generators without substantial equipment modification. COMs, which comprise a pulverized, comminuted or ground coal admixed with oil, may contain various additives to, for example, increase the wettability of the coal, stabilize the mixture, etc. This fuel mixture, while capable of being transmitted by pipeline, requires special handling and pumping equipment. These COMs have received extensive attention in the past decade but they are not new. U.S. Pat. No. 219,181, issued Feb. 24, 1879 to Smith, H.R. and Munsell, H.M. discloses the basic coal/oil mixtures and their use. COMs, while generally having a higher BTU content per unit volume than either coal or oil alone, have serious drawbacks. First, the oil used as the slurry medium draws from the U.S. domestic or foreign supply of crude oil; therefore, it only partially cuts down on this country's foreign oil dependence and reduces our balance of trade deficit. Second, there are severe restrictions on the export of oil even as a coal/oil mixture, thus there is a limited foreign market. Third, crude oil is expensive and, with the additional slurring expense, the cost savings to an oil-fired system are marginal. Finally, these COMs have all the inherent drawbacks of coal-containing slurries.

A further concept is the coal/liquid carbon dioxide slurry system. While high loading is possible, the trans-

port system requires cryogenics. They are expensive and involve a closed flow system requiring a return loop. Although coal/ liquid carbon dioxide slurries have not been altogether successful and require cryogenic pumping and handling systems, nevertheless, highly loaded liquid carbon dioxide slurries without the inherent drawbacks previously discussed would have viability. This would be especially true if the physical structure of the carbonaceous material were conductive to transport in a slurry and if such material were a uniform combustion product sufficiently high in BTU to offset the very high transport costs.

Thus it would be highly advantageous to have a fluidic fuel system which is easily and efficiently prepared from coal and which would be (a) transportable using existing cryogenic pipeline, tank car and tankship systems, (b) separable at the destination to provide a burnable, uniform carbonaceous material, (c) a uniform combustion product regardless of the region from which the coal is obtained, (d) high in BTU content per unit volume, (e) low in ash, sulfur and nitrogen, (f) high in solid loading and stability, (g) free of polluting process by-products which would have to be disposed of at the production site and (h) produced as part of a process which also yields a high quality liquid organic fraction which is pipeline transportable and can be used as a liquid fuel or as a quality feedstock material.

#### DISCLOSURE OF THE INVENTION

It has been discovered that a fluidic fuel system comprising a particulate coal char slurred in liquid carbon dioxide provides a pipeline transportable fuel composition which has high BTU per unit volume, is low in pollutants, and can be separated at the destination to provide a combustible solid as a combustion fuel. The by-product of the production of char is a high quality, liquid organic fraction which may be used in combustion devices or as a feedstock.

In the broad aspect of the invention, a liquid/solid mixture includes a particulate coal char portion dispersed in liquid carbon dioxide to create a composition which has fluidic characteristics such that it can be transported by certain cryogenic pipeline facilities. The mixture is separated and the particulate coal char is used as a fuel in char- or coal-fired combustion devices. The liquid organic material produced in forming the char is utilized as a feed stock or as a high quality liquid fuel for internal or external combustion devices. In a further aspect, that portion of char which is not slurred with the liquid carbon dioxide can be used directly as a feed for solid-fueled combustion devices. Preferably, the char is first admixed with a portion of the liquid organic material in order to enhance combustion, prevent absorption of moisture, increase the heat value of the char and reduce the danger of explosion.

In a further aspect, the particulate coal char can be admixed with raw coal, upgraded coal, petroleum coke and the like to yield a high BTU, reduced pollutant fuel for char- or coal-fired combustion devices. Likewise, the liquid organic fraction can be used itself as a fuel or admixed with a liquid petroleum distillate or lower and/or medium chain alcohols, such as those produced from grain, in order to vary the characteristics of the liquid as a fuel or as a feedstock.

The fuel composition of the instant invention can be produced by subjecting coal to pyrolysis or hydrolysis in the absence of oxygen to produce a particulate coal char which is admixed in suitable pro-

portions with liquid carbon dioxide to produce a solid-/liquid fluidic mixture, i.e., a slurry.

The liquid organic fraction is derived during the pyrolysis or hydropyrolysis of the coal. It may be further hydrogenated to alter the viscosity. Advantageously, the liquid organic fraction is beneficiated.

In accordance with one aspect of the invention, the fluidic fuel composition is produced by first subjecting coal to pyrolysis or hydropyrolysis in the absence of oxygen to produce a particulate coal char. The char is sized and otherwise mechanically and thermally treated to yield a particulate coal char of a distribution to advantageously effect loading of the solid. The liquid organic fraction obtained from the pyrolysis or hydropyrolysis of coal forms a completely combustible hydrocarbon-rich fuel suitable for pipeline transport and combustion directly in combustion systems and/or use as a chemical or refinery feedstock. Advantageously, this liquid organic fraction may be hydro-treated to reduce viscosity and beneficiated to remove sulfur or nitrogen pollutants.

In accordance with another embodiment, the liquid organic fraction is admixed with a lower chain alcohol which is preferably produced by well known synthetic methods utilizing coal and water or natural gas. In accordance with a greatly preferred embodiment, the alcohol is produced from the gases liberated in the pyrolysis process, thus producing all the fuel system components, except the liquid carbon dioxide, from a single, completely self-contained process system.

The utilization of a particulate char allows a high packing of the solid particulate matter for a given fluidity of the mixture. Thus, not only does one obtain the aforementioned advantages, but the energy requirement necessary to pump each BTU of fuel energy is reduced. In a further advantageous embodiment, the char is ground and sized to yield a particulate distribution which is bimodal or trimodal. The use of a bimodal or trimodal particulate char distribution enhances the packing of the solid.

In accordance with another embodiment of the instant invention, an amount of pulverized coal is added to the particulate coal char/liquid carbon dioxide slurry. In accordance with this embodiment, the coal is pulverized so as to provide bimodal or trimodal packing with the char. This improves the combustion characteristics of the solid fuel in some combustion applications without the expense of processing all the coal by pyrolysis. The amount of coal which is added is effective to improve the combustion characteristics without adversely affecting the beneficial aspects of the particulate coal char/liquid carbon dioxide mixture. Addition of coal to the slurry prior to transport is economically attractive in that grinding and sizing facilities at the slurry preparation site already exist.

In addition to the char and liquid organic fraction, the pyrolysis or hydropyrolysis produces gaseous products. These gases contain combustibles, lower chain hydrocarbons, hydrogen, carbon monoxide, ammonia, and sulfur and nitrogen compounds. The gases are useful for the extraction of marketable by products such as ammonia, and for use as a hydrogen source for hydropyrolysis, as a fuel for use in combustion systems and, most importantly, as a feedstock for the production of lower chain alcohols for use as viscosity modifiers for hydrocarbon liquids. Advantageously, the pyrolysis gases are "sweetened" prior to being marketed or used in the process. The elimination of potential pollutants in this

manner not only enhances the value of the char and liquid organic fraction as non-polluting fuels but also improves the economics of the process as the gaseous products may be captured and marketed or utilized in the process. In accordance with a preferred embodiment, these gases are used primarily to produce lower chain alcohols which are admixed with the liquid organic material to improve the viscosity characteristics of the liquid fraction.

10 In accordance with the instant invention, the particulate solid which is slurried to provide the transportation medium for the fuel to its end use, is separated from the liquid carbon dioxide by evaporation and injected directly into the combustion chamber of a combustion system in the presence of sufficient oxygen and heat to initiate and sustain combustion. The combustion products are then exhausted from the combustion chamber. In this manner, some or substantially all of the solid can be removed from the slurry and, either as the sole fuel 15 or in an admixture with coal, fired directly into solid-fueled combustion devices.

20 Further, in accordance with another aspect of the instant invention, the particulate char may be utilized, without slurring, directly for process heat and/or electric power generation. In a particularly preferred embodiment where the char and a liquid organic fraction are produced simultaneously by pyrolysis of coal, a portion of the liquid organic fraction, preferably a high boiling fraction, is admixed with the char in order to 25 enhance the heat value of the char, to prevent absorption of moisture, to facilitate combustion and to reduce 30 explosion hazard.

#### BEST MODE FOR CARRYING OUT THE INVENTION

35 In accordance with the preparation of the particulate coal char/liquid carbon dioxide slurry that is utilized in accordance with the instant invention, raw coal is continuously crushed to particles in the range of  $\frac{1}{2}$ " to  $\frac{1}{4}$ " in diameter to produce a crushed coal product. Advantageously, the crushed coal is then washed and otherwise beneficiated by means well known in the art to remove inorganics. This process and the size of the coal particle to be beneficiated will be dependent on the rank of the 40 coal, its agglomerating tendencies and the inorganic sulfur and ash content of the coal. The coal is preferably preheated to remove moisture and entrained gases which are advantageously used in the process. The crushed coal is then pyrolyzed or hydropyrolyzed 45 under temperatures and pressures and in accordance with process conditions to produce a particulate coal char. The thermal destructive distillation of the coal in the absence of oxygen to produce a coal char portion and a liquid organic fraction. Advantageously, the char portion may be further beneficiated to remove inorganic pollutants and mechanically and thermally treated to size the particulate char product which is 50 efficacious for bimodal and trimodal packing. The sized char mixture is then ready to be slurried.

55 60 The liquid organic fraction derived during the pyrolysis of the coal may be advantageously separated by fractional distillation into a higher boiling fraction containing the bulk of the nitrogen and a lower boiling fraction. The higher boiling fraction can be further 65 hydrogenated to decrease viscosity or sent to storage for use directly as a chemical reagent and feedstock. In accordance with one aspect, at least a portion of the higher boiling fraction is admixed with the char to form

an enhanced solid fuel for use, without slurring, directly in, for example, a mine mouth boiler. The lower boiling fraction is rendered substantially free of combined and entrained materials which, on combustion, would produce sulfur oxides, nitrogen oxides and like pollutants. The lower boiling fraction can be distilled to remove gasoline and other valuable hydrocarbon fractions which can be used directly as transportation fuels. The remaining lower boiling fraction is added to the upper boiling fraction.

The char is slurried with liquid carbon dioxide. The exact mixture of liquid to solid will depend on a number of factors such as the transportation medium limitations and the like. The transportable particulate coal char/liquid carbon dioxide slurry composition is passed to 15 cryogenic storage for later distribution by cryogenic pipeline or tanker vehicle.

The coals that can be employed in accordance with the instant invention are, generally, any coal which will undergo pyrolysis to form a particulate coal char. Preferably, coal from the lignite rank to the medium volatile bituminous have sufficient volatiles so as to maximize hydrocarbon production and minimize added water requirements. When lignites are utilized, they are advantageously subjected to pretreatment to remove residual water. This water is used as process water. Lignites are an advantageous starting material for the instant invention in that they contain process water for hydropyrolysis and/or process water as well as volatiles up to 55% by weight (on a dry basis). This is advantageous in obtaining the hydrocarbon-containing liquid organic fuel or feedstock.

The physical properties of the coal are also important in the practice of the instant invention. Those coals known as caking or agglomerating coals tend to form "cokes". Other coals of higher rank have plasticity and free swelling characteristics which tend to cause them to agglomerate and slake during the pyrolysis process. These coals must be subjected to special charring and treatment conditions as further set out herein to produce the particulate coal char suitable for use in accordance with the instant invention.

The mining and preparation of coal is fully described in Kirk-Othmer ENCYCLOPEDIA OF CHEMICAL TECHNOLOGY, second edition, Anthony Standin, editor, Interscience Publishers, New York, 1969, vol. 5, pp. 606-676. The coal is mined from a coal mine by either strip or underground methods as appropriate and well known in the art.

The raw coal is preferably subjected to preliminary crushing to reduce the particle size. Particle sizes of from  $\frac{1}{4}$ " to about  $\frac{1}{2}$ " in lateral dimension (diameter) are found useful but the actual sizing is dependent on the properties of the coal as well as the need for beneficiation. The need for size reduction and the size of the reduced material will depend upon the process conditions utilized as well as the composition and rank of the coal material. When beneficiation is necessary, for example, with coals containing a high percentage of ash or inorganic sulfur, the coal is preferably ground and subjected to washing and beneficiation techniques. When coals are used which have agglomerating tendencies, the size of the coal must be matched to the pyrolysis techniques and process conditions in order to produce a particulate coal char and to prevent slagging and/or agglomeration during pyrolysis. The crushing and/or grinding is preferably accomplished with impact mills such as counter-rotating cage mills, hammer mills or the

like. The crushed coal is sized by, for example, rough screening and gangue material is removed to assure a more uniform product for pyrolysis. Advantageously, carbonaceous fines and the like are readily utilized and subjected directly to pyrolytic destructive distillation.

In accordance with a greatly preferred embodiment, the crushed coal particles are then passed continuously through a preheater, which is operated in the range of from about 0.1 atmospheres to about 20 atmospheres and from about 100° C. to about 220° C. in order to remove gases and moisture. In many situations it has been found advantageous to employ a vacuum and/or mechanical manipulation to liberate moisture and gases in accordance with the instant invention. The moisture is advantageously used as process water for the hydropyrolysis and/or hydrotreating steps as further set forth herein. The entrained gases which are removed have further value as fuel or a hydrogen source for the hydropyrolysis step or as a feedstock for production of lower chain alcohols. Advantageously, the preheating is carried out using process heat from the char and hot gases liberated during pyrolysis. The preheating is preferably done at lower temperatures to avoid slagging and agglomeration.

Pyrolysis, as used herein, means the destructive distillation of coal in the absence of oxygen, and may be performed in the presence of one or more hydrogen donors or hydrogen itself. "Pyrolysis" thus includes pyrolysis, hydropyrolysis, and steam pyrolysis as well as carbonization techniques under varying temperature and pressure and atmosphere conditions such as, for example, in the presence of hydrogen, water vapor or hydrogen-donating material. The pyrolysis step of the instant invention can be carried out by any pyrolysis apparatus, which is well known in the art, having the ability to reach charring temperatures in the requisite time. For example, with subbituminous coals, temperatures should be in the range of from about 400° C. to about 800° C. and a heating rate of from about 1.5° C. per second to about 2.5° C. per second should be employed. Coals of higher rank require progressive heating at rates which prevent agglomeration and at higher final temperatures in the range of 1000° C. depending on the atmospheric pressures. It will be realized by the skilled artisan that, depending on the composition of the charge, the residence time, the pyrolysis process used and the charring furnace utilized, the temperatures and rates may vary. Preferably, the pyrolysis is performed in a continuous process.

As the crushed coal is heated in the absence of oxygen, the entrained materials are vaporized and collected. Lower boiling organic fractions including hydrocarbons, cyclics, and aromatics as well as higher boiling organic fractions are emitted from the coal leaving a particulate char material of essentially carbon which is of a porous structure and substantially spherical in shape. Included in the emitted constituents are the nitrogen containing polluting compounds such as pyridine, piperazine and the like.

The preferred method of thermal destructive distillation in the absence of oxygen is hydropyrolysis. Hydropyrolysis is advantageously employed when treating coal containing a lower percentage of volatiles or when a higher percentage of liquid organic material is desired. In accordance with this process, the pyrolysis is carried out in the presence of a hydrogen containing source which may be water or, advantageously, the pyrolysis

gases which are subjected to standard phase shift reactions.

The liquids hydrotreating step is quite well developed. A number of such technologies are readily available in the art. The parametric aspects of the pyrolysis conditions determine the char yield and the yield and composition of the liquids. Of the numerous pyrolysis technologies available, three are particularly applicable to the instant invention. They are a fluidized bed; an entrained flow reactor; and the pyrolysis/hydrotreater. The last is deemed preferable when the liquid organic fraction is to be further treated to adjust viscosity since it allows the sequential pyrolysis of coal and hydrotreating of the liquid.

In practicing the process of the instant invention in a continuous mode, it has been determined that recycling the hot char to the pyrolyzer conserves energy and has a beneficial effect on the pyrolysis products. The reactor temperature and the residence time are variable factors used to produce greater yields of char and/or liquid organic material, as well as obtaining a hydrocarbon mix of desirable viscosity. The process can be "fine tuned" depending on the rank of the coal (i.e., percent volatiles, agglomeration, etc.).

The char may be efficaciously sized and beneficiated. It is very important, in order to obtain the requisite liquid/ solid mixture, that the coal char be discrete, particulate char. When utilizing agglomerating or "caking" coals, preferably the process parameters are regulated so as not to produce an agglomerated product as previously set forth herein. Further, the coal char material may be emitted from the charring apparatus as discrete particles which are stuck together depending on the starting material and the pyrolysis conditions utilized. Therefore, the char material is ground to yield the substantially spherical, properly sized particulate coal char. Any conventional crushing and grinding means, wet or dry, may be employed. This would include ball grinders, roll grinders, rod mills, pebble mills and the like. Advantageously, the particles are sized and recycled to produce a desired distribution of particles. This is a very important aspect of the instant invention. The char particles are of sufficient fineness to pass a 100 mesh screen and the majority of the particles pass a 300 mesh screen. The mesh sizes refer to the Tyler Standard Screens. In accordance with the instant invention, char particles in the 100 mesh range or less are preferable. It will be realized that the particulate char of the instant invention having particle sizes in the above range is important to assure not only that the solid is high in reactivity, but also that the slurry is stable and can be pumped as a fluidic composition in cryogenic systems. The exact distribution of particle sizes is somewhat empirical in nature and depends upon the loading and stabilizers.

The ground, beneficiated char can be sized by any apparatus known in the art for separating particles of a size on the order of 100 mesh or less. Economically, screens or sieves are utilized, however, cyclone separators or the like can also be employed. In sizing, selections are made so as to assure a stable, pipeline transportable slurry and uniform combustion. A distribution of particle size is chosen to effect so called "model" packing. The spheroid shape of the primary particle provides spacing or voids between adjacent particles which can be filled by a distribution of second or third finer particle sizes to provide bimodal or trimodal packing. This modal packing technique allows addition of

other solid fuel material such as coal to the slurry without affecting the very advantageous pumping characteristics of the particulate coal char/liquid carbon dioxide slurry of the instant invention. Additionally, this packing mode allows the compaction of substantially more fuel in a given volume of fuel mixture while still retaining good fluidity.

The char may be beneficiated. When beneficiation is indicated because of the inorganics present, beneficiation may be utilized to clean either the coal or the char. The beneficiation can be performed by any device known in the art utilized to extract pollutants and other undesirable inorganics such as sulfur and ash. The char has a high degree of porosity which enables it to be readily beneficiated. Beneficiation may be accomplished, for example, by washing, jiggling, extraction, flotation, chemical reaction, solvent extraction, oil agglomeration (for coal only) and/or electro-static separation. The latter three methods remove both ash and pyritic (inorganic) sulfur. When the solvent extraction or oil agglomeration methods are used, it is most advantageous to utilize the liquid derived from the pyrolysis process as the beneficiating agent. The exact method employed will depend largely on the coal utilized in forming the char, the conditions of pyrolysis, and the char size and porosity.

The chars which can be utilized in accordance with the instant invention have a high reactivity and surface area, providing excellent Btu to weight ratios. The char particles are sufficiently porous to facilitate beneficiation and combustion but the pore size is not so large as to require the use of excessive liquid for a given amount of solid. The spherical shape allows adjacent particles to "roll over" one another, therefore improving slurry rheology and enhancing the solid loading characteristics. Preferably, chars that can be employed are discrete spherical particles which typically have a reaction constant of from about 0.08 to about 1.0; a reactivity of from about 10 to about 12; surface areas of from about 100 microns to about 200 microns; pore diameters of from about 0.02 milimicrons to about 0.07 milimicrons; and pass 100 mesh, and preferably, 200 mesh.

The resultant sized, particulate coal char mix may be conveyed by means of, for example, an air conduit to be "slurried" in appropriate proportion with liquid carbon dioxide.

The liquid organic fraction may be hydrotreated and/or beneficiated, as necessary, to provide a lower viscosity pollutant free organic fraction. The exact amount of this fraction utilized will depend upon the end-use properties desired. In accordance with a greatly preferred embodiment, the low boiling transportation fuels such as aviation gasoline, kerosene, naptha and the lighter diesel fuels are separated from the liquid organic fraction prior to transporting the liquid fraction when the liquids are to be used as a liquid fuel. These transportation fuels, which are pipeline transportable, can be marketed separately, thereby greatly improving the economics of the process.

The higher boiling fractions of the liquid organic fraction may contain certain sulfur and nitrogen compounds. This fraction may be removed by fractional distillation and used directly as a feedstock for chemical synthesis. Alternatively, it may be hydrotreated and beneficiated by methods well known in the art to reduce the viscosity and remove pollutants. Advantageously, the pyrolysis and hydrotreating can be accomplished

sequentially, followed by beneficiation in accordance with the procedure previously disclosed herein.

The particulate char and liquid carbon dioxide are admixed in the desired portion to form a slurry. An admixture is thus formed of a particulate coal char and liquid carbon dioxide having a ratio of particulate char to liquid which is dependent upon the properties of the slurry desired.

The terms "slurry" or "liquid/solid mixture" as used herein are meant to include a liquid carbon dioxide composition containing an amount of the particulate coal char. For most applications, however, the particulate coal char constituent should comprise not less than about 45% by weight of the composition and preferably from about 70% to about 90% by weight.

In accordance with another aspect of the instant invention, the particulate char is admixed with an amount of liquid organic material effective to reduce absorption of the liquid carbon dioxide by the char and to enhance the combustion characteristics of the fuel. This treatment serves to prevent absorption by the particulate char of an excess of the liquid carbon dioxide. The greater the absorption of carbon dioxide by the particulate char, the greater the retention by the char particles after separation. This retention of non-combustible carbon dioxide not only impedes combustion but also removes gas from the return cycle which must be made up. When absorption rates by the char are in excess of about 7%, pretreatment is very beneficial. It will be realized that absorption of the liquid carbon dioxide by the char impedes combustion of the fuel.

In accordance with this pretreatment, the char is brought into intimate contact with an amount of a the coating material effective to reduce the absorption of liquid by the char and to enhance the combustion characteristics. The treatment is effected prior to the particulate char being slurried with the liquid. The coatings that are useful include organic and inorganic materials which will not produce pollutants upon combustion. Since surfactants and emulsifiers are used to enhance slurry stability, care must be taken that the coating is compatible with the stabilized composition. Coating materials which are particularly advantageous include parafins and waxes as well as the longer chain aliphatics, aromatics, polycyclic aromatics, aro-aliphatics and the like. Mixtures of various hydrocarbons, such as #6 fuel oil, are particularly desirable because of their ready availability and ease of application. Advantageously, the higher boiling liquid organic fractions from the pyrolysis of the coal are utilized. The sealant or coating can be applied to the char by spraying, electrostatic deposition or the like.

In accordance with another aspect of the instant invention, a portion of the char produced by pyrolysis of coal can be used directly, without slurring, as a solid combustion fuel. Preferably, the char which is not slurried is admixed with a portion of the hydrocarbon liquid, enhancing combustion but maintaining the char substantially as a particulate solid matter, i.e., not a fluidic mixture. In this embodiment, preferably the higher boiling "tar" fractions are used. These fractions adhere well to the hot char and provide a "sealant" to prevent moisture absorption during transport. They are also high in heat value per unit volume.

In accordance with another embodiment of the instant invention, coal, or more preferably the pyrolysis gases, and water are utilized to produce methanol and other lower chain alcohols which are utilized to en-

hance the viscosity of the organic liquid. Water released from the coal during preheating can be used as part of the water required in the synthesis.

As used herein the term alcohol is employed to mean alcohols (mono-, di- and trihydroxy) which contain from 1 to about 4 carbon atoms. These include, for example, methanol, ethanol, propanol, butanol and the like. The alcohol may range from substantially pure methanol to various mixtures of alcohols as are produced by the catalyzed reaction of gases derived from pyrolysis or natural gas. Advantageously, the alcohol constituent can be produced on site at the mine in conjunction with the pyrolysis. The process heat can be supplied from the cooling of the pyrolysis products.

In accordance with the process for making these alcohols directly from coal and steam, carbon monoxide and hydrogen are initially formed in accordance with equation I:



A portion of the gas is subjected to the shift reaction with steam to produce additional hydrogen in accordance with equation II:



The  $CO_2$  is scrubbed from the gaseous product leaving only hydrogen. The hydrogen is admixed with gaseous products of equation I to produce a gas having desired ratio of hydrogen to carbon monoxide from which methanol and similar products are synthesized catalytically. Preferably, the gas having the desired ratio of hydrogen to carbon monoxide is produced during the coal pyrolysis, and more preferably by hydropyrolysis.

In accordance with this aspect of the instant invention, the raw pyrolysis gas which contains water vapor is subjected to sulfur and nitrogen removal as previously disclosed. The  $H_2$  and  $CO$  are then separated by, for example, cryogenic means and converted to methane. The methane, ethane and higher hydrocarbon gases are converted to the alcohols.

In the methanol synthesis plant the respective constituents, such as carbon monoxide and hydrogen, are combined to produce methanol. The synthesis of methanol is described in pages 370-398 of vol. 13 of the above referenced KIRK-OTHMER ENCYCLOPEDIA. The carbon monoxide and hydrogen are controlled in a ratio and temperature pressure combination to obtain maximum yields of the methanol fuel product. Other methods for methanol synthesis at lower temperatures and pressures are also known, as for example, the ICI low pressure process as described in "Here's How ICI Synthesizes Methanol at Low Pressure", Oil and Gas Journal, vol. 66, pp. 106-9, Feb. 12, 1968. In accordance with this aspect of the instant invention, the alcohol is used as a portion or substantially all of the liquid phase in the slurry.

In accordance with another aspect of the instant invention, the particulate char solid can be supplemented by an amount of particulate carbonaceous material such as coal, effective to improve combustion characteristics without detrimentally affecting the beneficial aspects of the uniform combustion slurry product. Specifically, applicant has disclosed that coal-liquid carbon dioxide mixtures contain coal and, therefore, suffer many of the drawbacks of coal-containing slurries. In accordance with the instant invention, it has been found that certain amounts of particulate coal can be added to the particu-

late coal char/liquid carbon dioxide slurry with beneficial effect. Coal, as used in this aspect, means raw coal of bituminous, subbituminous and anthracite rank as well as upgraded coals, petroleum coke and the like. Preferably, coals containing higher ash and inorganic sulfur are beneficiated by methods disclosed hereinbefore prior to their introduction into the slurry. Upgraded coals include those which have been thermally dried or compressed under heat and mechanical pressure to effect a slight carbonization of the coal (so-called carbonized coal) such as K-Fuel® (process disclosed in U.S. Pat. No. 4,052,168). Surprisingly, where the coal is properly sized and "packed" with the particulate char, the rheology characteristics of the particulate coal char/liquid carbon dioxide slurry are not greatly affected. Practice of the invention in accordance with this embodiment is advantageous when firing into combustion systems in which char, because of its higher ignition point, is not fully combusted. The coal ignition helps to raise the temperature of certain combustion system configurations to facilitate char ignition. Additionally, use of pulverized coal is economically advantageous in that the coal portion of the slurry does not have to undergo pyrolysis. The amount of coal that can be used in accordance with the invention will depend on the particular properties of the coal, but for many applications, up to 50% by weight of the solid constituent of the slurry can be coal and advantageously up to about 30% by weight of the solid.

The liquid carbon dioxide is prepared by subjecting gaseous CO<sub>2</sub> to pressure in the absence of heat in accordance with standard cryogenic procedures. The mixing (or slurring) of the solid particles and the liquid carbon dioxide can be accomplished by methods developed for slurring coal in liquid carbon dioxide. As previously set forth, the sizing and packing of the slurry is particularly important in obtaining a highly loaded, stable, transportable combustion fuel. It has been found advantageous to have greater than about 50% of the solid material smaller than about 100 mesh (Tyler) and over about 80% of that passing a mesh size in the range of 300 (Tyler).

The high BTU, non-polluting fluidic fuel system, upon reaching its ultimate destination, is separated so that substantially all of the solid portion of the slurry is removed from the liquid carbon dioxide. This is accomplished by decanting followed by depressurization, i.e., evaporation. After separation, the solid component can be used as a fuel for solid-fueled combustion systems.

The separated char (or carbonaceous material/char mixture if carbonaceous material has been added to the slurry system) can be burned alone or with a mixture of particulate carbonaceous material such as raw coal, upgraded coals, coke, petroleum coke or the like in standard solid-fueled combustion systems. By admixing the char with one or more of these carbonaceous materials, a high quality compliance product can be obtained even if the admixed material is low in BTU and/or high in sulfur.

It will be realized that the liquid organic fraction when used as a fuel, can be combusted alone or combined with liquid petroleum distillates as previously disclosed and/or lower to medium chain alcohols having from 1 to about 10 carbon atoms, such as those produced from grain or bio-waste synthesis processes or the raw gas as previously described, to enhance certain fuel characteristics for a particular application.

In accordance with a further aspect of the instant invention, the solid particulate char which is not admixed with liquid carbon dioxide to form the slurry can be used independently as a fuel for combustion devices. 5 In accordance with this aspect, some or a substantial portion of the char produced in pyrolysis or hydropyrolysis can be used directly as a fuel for solid-fueled combustion devices. The char to be fired directly as a solid fuel need not be ground or sized. It may be 10 mixed with other particulate carbonaceous material and transported to the end-use destination by rail car, truck or the like. Advantageously, the char is transported pneumatically. In a particularly advantageous embodiment, the hot char is fed directly to a mine mouth combustion system, either with or without the addition of coal, upgraded coal and the like. Preferably, this is accomplished by means of a pneumatic conveyance device. In accordance with a further aspect of this embodiment as previously set forth herein, an amount of 15 20 the liquid organic material which is effective to enhance combustion characteristics, reduce explosion hazard, and prevent moisture absorption is admixed with the char. Preferably, the higher boiling hydrocarbon liquid fractions are used. This helps to reduce the viscosity of 25 the remaining liquid organic material.

In this aspect of the invention, the higher boiling fraction of the liquid organic material is used to admix with the char and some or a substantial portion of the remaining liquid organic material may be used as a 30 liquid fuel. As previously described, certain lower boiling fractions such as gasoline and distillates are removed for use directly as transportation fuels. These fuels are transported in the pipeline by use of plugs and the like to refineries or to combustion systems requiring 35 high grade fuels. A substantial portion of the liquid organic material is economically transported by means of, for example, tanker truck for use directly as a fuel for liquid-fueled combustion devices or as a feedstock. It will be realized that the liquids can first be "cracked" or 40 hydrotreated to enhance their value as a fuel.

Combustion systems designed for burning coal will utilize the fuel system of the instant invention most readily. Char has a higher ignition point than coal but is more reactive. It will be realized by the skilled artisan that modification to coal-fired systems may be necessary to avoid boiler derating if the fuel system of the instant invention is fired directly into the combustion system.

Char- or coal-fired combustion devices, with little or 50 no modification, can burn the particulate coal char portion of the slurry which serves as the solid component of the fuel system. Coal, either carried in the fluidic fuel system or added to the char after separation will allow a "tuning" of the solid fuel to any coal-fired combustion system. Because the char is beneficiated, coals of higher sulfur and/or lower BTU can be blended with the char to effect a compliance mixture with no derating of the boiler system.

It will be further realized that the fuels of the instant 60 invention, either individually or in combination, can be combusted in combustion devices using oxygen. Oxygen, as that term is used herein is intended to include atmospheres of pure oxygen as well as atmosphere having a partial pressure of oxygen such as, for example, air.

A particularly advantageous aspect of the instant invention relates to the flexibility of the instant transportable fuel system. The transportable fuel system can

be "adjusted" or "fine tuned" during the process, prior to transportation or at the end-use facility. The system of the instant invention facilitates transporting coal-derived fuels to both liquid fueled and solid fueled combustion systems as well as providing a useful hydrocarbon feedstock. The fuel is uniform and non-polluting. The components can be beneficiated to remove harmful constituents, thus avoiding the SO<sub>2</sub> and NO<sub>x</sub> pollutants linked with acid rain as well as ash related boiler slagging problems. There is no preclusion against exporting the slurry or the liquid organic material and export of the liquid is accomplished using cryogenic transportation systems. The fuel system utilizes all ranks of coals, including lower ranks and coals not previously thought economically viable. Most importantly, unlike coal, the solid fuel is a uniform combustion product.

While the invention has been explained in relation to its preferred embodiment it is understood that various modifications thereof will become apparent to those skilled in the art upon reading the specification and the invention is intended to cover such modifications as fall within the scope of the appended claims.

We claim:

1. A fluidic, substantially non-polluting fuel transportation system comprising a liquid/solid mixture, including a portion of a particulate coal char, dispersed in an amount of liquid carbon dioxide effective to produce a transportable composition, wherein substantially all of the solid portion is separated at the destination for use as a solid fuel.

2. The fuel system of claim 1 further comprising a portion of a particulate carbonaceous material selected from the group consisting of raw coal, upgraded coal, petroleum coke and mixtures thereof.

3. The fuel system of claim 1 wherein the solid portion is beneficiated and treated to effect bimodal or trimodal packing thereof.

4. The fuel system of claim 2 wherein the solid portion is beneficiated and treated to effect bimodal or trimodal packing thereof.

5. The fuel system of claim 1 wherein the solid is at least partially derived by the pyrolysis of coal.

6. The fuel system of claim 1 wherein said particulate coal char is treated with an amount of a coating effective to reduce absorption of liquid carbon dioxide and to enhance the combustion characteristics of the char.

7. The fuel system of claim 6 wherein said coating comprises at least a portion of the higher boiling fraction of the liquid organic fraction produced by the pyrolysis of coal.

8. A method of producing a substantially non-polluting fluidic fuel transportation system comprising the steps of admixing a particulate coal char with an amount of liquid carbon dioxide effective to produce a transportable liquid/solid mixture; transporting said transportable liquid/solid mixture; and separating from said transportable liquid/solid mixture substantially all of said solid for use as a fuel.

9. The method of claim 8 comprising the further step of admixing with said liquid/solid mixture prior to said transporting step a portion of a particulate carbonaceous material selected from the group consisting of raw coal, upgraded coal, petroleum coke and mixture thereof.

10. A method for producing a substantially nonpolluting fluidic fuel transportation system comprising the steps of

- (a) subjecting coal to pyrolysis to produce a coal char, a liquid organic material and a hydrocarbon containing gas;
- (b) treating a coal char to produce a particulate coal char;
- (c) admixing said particulate coal char and liquid carbon dioxide to form said fluidic fuel transportation system;
- (d) transporting said system to a destination; and
- (e) removing from said system substantially all of said solid for use as a fuel.

11. The method of claim 10 wherein said pyrolysis is hydropyrolysis and is carried out in the presence of compounds selected from the group consisting of water, hydrogendonating compounds, hydrogen and mixtures thereof.

12. The method of claim 11 further comprising the steps of beneficiating said liquid organic material and said solid.

13. The method of claim 11 further comprising a preheating step at temperatures in the range of from about 100° C. to about 220° C. at pressures of from about 0.1 atmospheres to about 20 atmospheres prior to said pyrolysis step and a presoaking step in the presence of a steam atmosphere at atmospheres of from about 40 to 60 atmospheres and at temperatures in the range of from about 200° C. to 400° C. subsequent to said preheating step but prior to said pyrolysis step.

14. The method of claim 10 further comprising the step of admixing a portion of a particulate carbonaceous material selected from raw coal, upgraded coal, coke, petroleum coke and mixtures thereof with said coal char prior to said admixing step.

15. The method of claim 10 further comprising the step of coating the solid prior to said admixing step with an amount of a coating material effective to substantially diminish the absorption of said liquid carbon dioxide.

16. The method of claim 15 further comprising the step of coating the solid prior to said admixing step with an amount of a coating material derived from said liquid organic material effective to substantially diminish the absorption of said liquid carbon dioxide by said solid and to enhance the combustion characteristics thereof.

17. The method of claim 16 wherein said coating comprises the higher boiling fraction of the liquid organic material derived simultaneously with the char from the pyrolytic destructive distillation of coal.

18. A method of firing a combustion device comprising the steps of:

- (a) injecting a combustible amount of a fuel composition into a combustion chamber wherein said fuel composition is selected from a group consisting of
  - (1) a solid material of particulate coal char obtained from removal of at least a portion of the solid of a liquid/solid mixture including a portion of a particulate coal char, dispersed in an amount of liquid carbon dioxide effective to produce a transportable composition;
  - (2) a solid coated material of particulate coal char admixed with an amount of the liquid organic material effective to substantially reduce absorption of liquid carbon dioxide and to enhance combustion, such solid coated material being obtained from removal of at least a portion of the solid portion of a liquid/solid mixture including a portion of a coated solid material dispersed in

- an amount of liquid carbon dioxide effective to produce a transportable composition;
- (b) admixing said combustible amount of said fuel composition with sufficient oxygen to support substantially complete combustion, thus producing a totally combustible mixture;
- (c) heating said combustible mixture to the ignition point;

- (d) sustaining the combustion within said chamber; and
- (e) exhausting the combustion by-products from the chamber.

5 19. The method of claim 18 wherein said solid further comprises an amount of a carbonaceous material selected from raw coal, upgraded coal, petroleum coke and mixtures thereof.

\* \* \* \* \*

10

15

20

25

30

35

40

45

50

55

60

65